

# UNITED STATES PATENT OFFICE

ROBERT ABBOTT HADFIELD, OF WESTMINSTER, ENGLAND.

## MANUFACTURE OF MANGANESE STEEL.

1,310,528.

Specification of Letters Patent. Patented July 22, 1919.

No Drawing.

Application filed August 10, 1917. Serial No. 185,521.

*To all whom it may concern:*

Be it known that I, Sir ROBERT ABBOTT HADFIELD, Bart., F. R. S., a subject of the King of Great Britain and Ireland, residing at Westminster, England, have invented Improvements in or Relating to the Manufacture of Manganese Steel, of which the following is a specification.

This invention relates to the manufacture of steel of the kind comprising as its main constituents iron, manganese, carbon and silicon, and in which the proportion of manganese is high as in steel of the kind known as manganese steel.

In the manufacture of manganese steel it has heretofore been usual to add ordinary ferro-manganese containing about 80% manganese to decarbonized and desiliconized iron in such proportion that, after allowing for a certain amount of oxidation, the resulting manganese steel contains usually about 11 $\frac{1}{2}$  to 14 per cent. of manganese, the carbon present amounting to about 1.2 to 1.4 per cent. and silicon being usually kept as low as possible, very seldom exceeding about .25 to .3 per cent.

Now the present invention has for object to produce a manganese steel possessing qualities that will render it, particularly when in the form of plates or sheets, better adapted for some purposes, particularly as a protective material against bullets, pieces of shrapnel and like missiles, than ordinary manganese steel.

Now I have found that this desirable object can be attained by increasing the percentage of silicon in the steel by purposely adding silicon to the materials used for making manganese steel. Good results can be attained with the silicon within the limits of from about .65 to 2.5% the carbon being within limits of from about .90 to 1.25% and manganese within the limits of from about 10 to 17%. The new product seems somewhat tougher with lower carbon and yet its hardness is not so much or only slightly reduced by the lower percentage of carbon. The carbon may however in some cases be increased to a higher percentage, say for example to 1.5% or even to 2%, especially when the steel is not to be rolled but used in the form of castings, and it may be reduced to .75% or even lower. The lower limit of carbon present in the new steel is however not confined to the percentage mentioned but the upper limit should not exceed

about 2% and will usually be much lower. The percentage of carbon is therefore comparatively low compared with the manganese as in ordinary manganese steel. The main feature of the new steel is the presence therein of a relatively high percentage of silicon as compared with ordinary manganese steel of commerce. Such a manganese steel, which may be called for distinction, high silicon manganese steel, is found, after being specially toughened in the manner usually adopted for toughening manganese steel, namely by heating it to a high temperature and quenching it in water, to possess greater toughness and resistance to perforations than ordinary manganese steel and therefore when rolled into plates or sheets, to offer greater resistance to perforation by bullets and other missiles than ordinary manganese steel of the same thickness.

The toughening of the new steel may be effected by heating it to a temperature say for example of about 900° C. and up to, it may be, about 1050° C., or even above but below its melting point and quenching it in water.

The new or high silicon manganese steel can conveniently be produced by adding silicon to a mixture of iron and ferro-manganese which may be the ordinary 80% ferro-manganese of commerce. The silicon may be added as such or in any other suitable or convenient form, as for example ferro-silicon or silicon spiegel, conveniently the latter, the proportion of the ingredients used being such as to produce a steel containing a high manganese content, say of the order of 10 to 17 per cent. about .6 to 2 per cent. of silicon and about .75 to 2 per cent. of carbon. The resulting steel may be cast into ingots or other castings.

For many purposes, the new manganese steel may advantageously be rolled into the form of sheets or plates (hereinafter referred to as sheets), or rods, bars or wire, before or after being subjected to the toughening process referred to. If desired, the toughening process may be repeated. The new manganese steel can also be used for castings of any desired shape and be heat treated or not as may be required, according to the purpose for which it is to be used.

The following are given as examples of high silicon manganese steels according to the invention that have been found, after being specially toughened as described and

rolled into sheets to give satisfactory results as a protective material for use in the construction of helmets, body shields and protective armor for air craft namely:

| 5      | Fe    | C     | Si     | Mn |
|--------|-------|-------|--------|----|
| 84.89% | 1.04% | 1.42% | 12.65% |    |
| 85.20  | 1.00  | .65   | 13.15  |    |

Aluminium may be added to the new steel. 10 Or the silicon in the new manganese steel may be replaced in whole or in part by aluminium which appears to be its equivalent for some purposes, as for the purpose of increasing the toughness of the resulting 15 manganese steel and its resistance to perforation. Thus, the new steel may contain for example about equal parts of silicon and aluminium, say for example .75% of each. The claims as hereunto appended 20 while mentioning only silicon are to be understood as covering such equivalent.

The quality of the new manganese steel can be further varied or improved by the addition thereto of another element such for 25 example as chromium, nickel, cobalt, vanadium, tungsten or titanium or of two or more of such elements the percentage of such element or elements employed being such say for example from one half of one per cent. to seven per cent. as to give the varying desired qualities to the resulting steel 30 or alloy.

One example of the new steel with addition of chromium that has been found to 35 possess excellent qualities after toughening by heating and cooling as described and rolling into plate or sheet form is as follows:—

| 40 | Fe     | C     | Si    | Mn     | Cr   |
|----|--------|-------|-------|--------|------|
|    | 84.08% | 1.04% | 1.42% | 12.65% | .81% |

It is to be understood that the use of the new manganese steels hereinbefore described is not limited to the manufacture of sheets for protective purpose as they may be found 45 useful for various other purposes and in either the rolled or cast condition.

What I claim is:—

1. The herein described process of producing steel of great toughness and resistance which consists in adding silicon to and melting it with manganese steel so as to increase the content of silicon therein from about decimal six of one per cent. to two decimal five per cent., heating the resulting 55 high silicon manganese steel to a high temperature below its melting point and afterward quenching it in water.

2. The herein described process of producing steel of great toughness and resistance which consists in adding to manganese steel containing in addition to iron, carbon up to about two per cent., and from about 60 ten to seventeen per cent. of manganese,

silicon so as to increase the content thereof 65 in the steel to about decimal six of one per cent. to two decimal five per cent., heating the resulting high silicon manganese steel to a high temperature below its melting point and quenching it in water. 70

3. The herein described process of producing steel of great toughness and resistance which consists in adding to manganese steel containing in addition to iron, carbon up to about two per cent., and from about 75 ten to seventeen per cent. of manganese, silicon so as to increase the content thereof in the steel to about decimal six of one per cent. to two decimal five per cent., casting the resulting high silicon manganese steel 80 into an ingot, converting said ingot into a desired shape and thickness by appropriate means, heating the said steel to a high temperature below its melting point and cooling it quickly.

4. The herein described process of producing steel of great toughness and resistance which consists in adding to manganese steel containing in addition to iron, from about decimal seven of one per cent. to two 90 per cent. of carbon and from about ten to seventeen per cent. of manganese, silicon so as to increase the content thereof in the steel to from about decimal six of one per cent. to two decimal five per cent., converting the resulting high silicon manganese steel into a thin body, heating the said body to a high temperature below its melting point and afterward cooling it quickly. 95

5. The herein described process of producing steel of great toughness and resistance which consists in adding to manganese steel containing in addition to iron from about decimal seven of one per cent. to two 100 per cent. of carbon, and from about ten to seventeen per cent. of manganese, silicon so as to increase the content thereof in the steel to from about decimal six of one per cent. to two decimal five per cent., converting the resulting high silicon steel into a 110 sheet, heating such sheet to a high temperature below its melting point and quenching it in water.

6. As a new article of manufacture, wrought manganese steel possessing great 115 toughness and resistance to perforation and containing iron with from about decimal seven of one per cent. to one decimal five per cent. of carbon, from about ten to seventeen per cent. of manganese and from about decimal six of one per cent. to about two decimal five per cent. of silicon. 120

7. As a new article of manufacture, wrought manganese steel possessing great 125 toughness and resistance to perforation and containing iron with about one per cent. of carbon, from about ten to fourteen per cent. of manganese and from about decimal six

of one per cent. to one decimal six per cent. of silicon.

8. As a new article of manufacture, wrought manganese steel in sheet form possessing great toughness and resistance to perforation and containing iron with from about decimal seven of one per cent. to one decimal five per cent. of carbon, from about ten to seventeen per cent. of manganese and from about decimal six of one per cent. to one decimal six per cent. of silicon.

9. As a new article of manufacture, wrought manganese steel in sheet form possessing great toughness and resistance to perforation and containing iron with about one per cent. of carbon, from about ten to fourteen per cent. of manganese and from

about decimal six of one per cent. to one decimal six per cent. of silicon.

10. As a new article of manufacture, wrought manganese steel in sheet form possessing great toughness and resistance to perforation and containing iron with about one per cent. of carbon, about twelve to thirteen per cent. of manganese and from about decimal six of one per cent. to one decimal five per cent. of silicon.

Signed at 22 Carlton House Terrace in the city of Westminster, England, this twelfth day of July 1917.

ROBERT ABBOTT HADFIELD.

Witnesses:

WILLIAM CROSS,  
LEONARD ROWLAND.